

July 14, 1925.

W. H. SMITH ET AL.

1,545,705

ALLOY AND METHOD OF MAKING AND CASTING SAME

Filed Aug. 22, 1921

Fig.1.



Fig. 2.



Fig. 3.



Fig. 4.



INVENTORS.

BY William H. Smith  
Charles M. Campbell

*William H. Smith*  
ATTORNEY.

Patented July 14, 1925.

1,545,705

# UNITED STATES PATENT OFFICE.

WILLIAM H. SMITH, OF EAST CLEVELAND, AND CHARLES M. CAMPBELL, OF CLEVELAND, OHIO, ASSIGNEES TO THE PIONEER ALLOY PRODUCTS COMPANY, OF CLEVELAND, OHIO, A CORPORATION OF DELAWARE.

## ALLOY AND METHOD OF MAKING AND CASTING SAME.

Application filed August 22, 1921. Serial No. 494,055.

To all whom it may concern:

Be it known that we, WILLIAM H. SMITH and CHARLES M. CAMPBELL, residing, respectively, at East Cleveland and Cleveland, in the county of Cuyahoga and State of Ohio, have invented a certain new and useful Improvement in Alloys and Methods of Making and Casting Same, of which the following is a full, clear, and exact description, reference being had to the accompanying drawings.

This invention relates to apparatus for technical chemical operations such as are encountered in acid works, alkali works, oil refineries, dye works, steel works, general chemical manufacturing, electrolytic works and numerous other places in the arts where valves, cocks, pipes, fittings, pumps, containers, evaporators, condensers, concentrators, mixing machines and other devices are employed. The ultimate object of the invention is the provision of an intrinsically inexpensive metal or alloy for these purposes which shall be sufficiently resistant to corrosion to exhibit a long life, which shall be sufficiently strong mechanically to withstand the ordinary usage to which such devices are subjected, and which shall be easily machined, forged, or otherwise fabricated. No material having all these qualities has ever come into commercial use, although materials possessing some of these qualities have long been known. For example, platinum is nearly perfect excepting for its cost; glass and porcelain having the necessary chemical resistivity but are mechanically fragile and also difficult to work. Numberless alloys exist having the necessary strength and workability but deficient in chemical resistivity.

It has long been suspected that some alloy containing essentially chromium and one or more iron group metals could be employed for this purpose, but no one has heretofore produced either a composition or a mode of handling it which resulted in a product of the highest utility from the chemical standpoint, the chief difficulty being that an admixture of any material amount of carbon renders such an alloy unworkably hard, physically brittle, and chemically non-resist-

ant. However, between this previous methods of producing such alloys have always resulted, at least when performed on a commercial scale, in the absorption of such an amount of carbon as to render the product of very small value for chemical apparatus regardless of whether an open hearth furnace, crucible furnace, or electric furnace be employed. A bath containing any material amount of molten chromium will dissolve solid carbon from fuel or crucible, carbon gas such as hydrocarbon or monoxide from combustion products, or volatilized carbon from an electric arc with equal avidity. Heretofore alloys containing more than about 20% of chromium have been considered practically unmanageable.

The immediate objects of this invention are the provision of a furnace charge and a mode of manipulation which shall result in a useful, low-carbon, alloy, containing essentially the ingredients named, with or without other ingredients; the provision of a furnace charge containing the essential substances in their cheapest and most available forms; the provision of a furnace charge and mode of manipulation such as shall facilitate the fusion and enable the operation to be conducted at the lowest possible temperature; the provision of a new and improved slag for alloys of this nature; while further objects and advantages of the invention will appear as the description proceeds.

In the drawings, Fig. 1, is a view showing the charge prior to melting, and Fig. 2 shows the same charge melted; Fig. 3 illustrates the mold, and Fig. 4 certain apparatus made of alloy.

It is necessary to employ an electric furnace and this of a type wherein all the electric terminals are located above the surface of the metal bath. The hearth of the furnace is preferably made of magnesite and all carbon or carbonaceous matter is kept away from it. We preferably mix it with hydrochloric acid instead of the usual molasses, and mold the mixture into the desired form, afterwards sintering the hearth in any mode customary in electric furnace practice. This operation serves to contam-

inate the magnesite with a certain amount of carbon which must now be removed and this we effect as by introducing a small amount of low carbon iron scrap together with lime and enough fluorspar to thin the slag. The furnace interior is thoroughly washed as many times as is necessary to bring the hearth to a neutral condition as regards the absorption of iron and the evolution of carbon, this condition being ascertained by analyzing the metal poured off. This slag is also very effective in removing all silica and compounds thereof.

A specimen charge is as follows:

|    |                            |           |
|----|----------------------------|-----------|
| 15 | Ferrochrome (.40% C.)      | 35. lbs.  |
|    | =Fe 10.                    |           |
|    | Cr 24.86                   |           |
|    | C 0.14                     |           |
| 20 | Iron (.14% C.)             | 25. lbs.  |
|    | Fe 24.96                   |           |
|    | C .04                      |           |
|    | Nickel (free from carbon)  | 30. lbs.  |
| 25 | Ferro-molybdenum (1.0% C.) | 10. lbs.  |
|    | Fe 4.9                     |           |
|    | Mo 5.                      |           |
|    | C 0.1                      |           |
|    |                            | 100. lbs. |

In terms of totals this charge contains approximately: chromium 25, iron 40, nickel 30, molybdenum 5, carbon .28.

Inasmuch as the iron content of ferrochrome and ferro-molybdenum is quite variable it is impossible to predict a charge with accuracy in terms of these ingredients, although considerable latitude in ultimate composition is permissible. In general we preferably adjust the proportions of these ingredients in accordance with their composition so as to secure a charge lying substantially within the range indicated by the following:

|                    | A  | B  | C  | D  | E  | F   | G   | H  |
|--------------------|----|----|----|----|----|-----|-----|----|
| Chromium           | 20 | 20 | 25 | 25 | 30 | 30  | 35  | 35 |
| Nickel (or cobalt) | 35 | 40 | 30 | 40 | 25 | 30  | 30  | 40 |
| Iron               | 40 | 35 | 40 | 30 | 40 | 35  | 30  | 22 |
| Molybdenum         | 5  | 5  | 5  | 5  | 5  | 5   | 5   | 8  |
| Carbon below about | .3 | .3 | .3 | .3 | .3 | .25 | .25 | .2 |

The higher the chromium and the lower the nickel the less the carbon content must be in order to avoid brittleness and low chemical resistivity.

We do not restrict ourselves to the charge specified as we may omit the nickel entirely, replacing it with either cobalt or iron, and may vary the chromium content through a wide range. Indeed in the absence of nickel (or cobalt) an increased amount of chromium is necessary to secure chemical resistivity. We have used

with success a charge containing approximately:

|            |        |
|------------|--------|
| Chromium   | 50     |
| Iron       | 44-1/2 |
| Molybdenum | 5-1/2  |

resulting in an alloy of approximately:

|            |       |
|------------|-------|
| Chromium   | 45-47 |
| Iron       | 50-48 |
| Molybdenum | 5     |

This alloy is extremely difficult to make owing to its great avidity for carbon, and to the necessity for keeping the carbon below .2% and preferably even lower. This requirement necessitates the use of a purer grade of ferrochrome which increases its expense disproportionately, and the melting point is inconveniently high. The use of nickel avoids all these drawbacks, yet the ternary alloy just mentioned is very satisfactory in use and can be made successfully by the process herein described.

The iron is thrown or piled in the center of the hearth as shown at A in Fig. 1, the nickel (when used) around it, as shown at B, the ferrochrome around that, as shown at C, that last being kept out of contact with the electrodes and covered with a mixture of lime and fluorspar D, some three or four inches deep. This lime and fluorspar must be of good quality, mixed thoroughly together in the proportion of about 80% to 90% of lime and the balance fluorspar, the two being preferably ground together to a condition of inseparable intermingling. Silica and its compounds are excluded both because of the danger of reduction by chromium and the certainty that the melting point of the slag would be unduly decreased. The molybdenum is not added until the last. Indeed it is possible and highly satisfactory to add only the iron at first and follow with the other ingredients but the mode described is quicker and more convenient.

The furnace is then started in the usual manner, and as soon as the iron has melted the heat thereof slowly causes the ferrochrome to dissolve therein and the slag to soften and flow thereover, so that the arc can no longer strike through the slag into contact with the molten mass. This is rendered possible by the fact that this slag becomes conducting under the temperature of the electric arc. This covering of the bath with the slag must be effected by the time the ferrochrome begins to melt, else the same will absorb carbon from the arc, but the iron and nickel will not do so. When the entire charge has been melted and incorporated thoroughly together, a suitable deoxidizer is added and the molybdenum or ferro-molybdenum or other added substance is incorporated, after which the alloy is

drawn and poured. Prior to pouring, however, the temperature of the furnace must be raised considerably, since the best pouring temperature is very high (about 3200° F.)

At all times a complete layer of slag must be maintained over the metal, especially between it and the electrodes, and this is effected by maintaining its composition high in lime and low in all substances of a low melting point such as fluorspar and silica or compounds thereof. With a lime content of 80% to 90% the space under each electrode will constitute a kind of crater but its bottom will consist of a layer about one fourth inch in thickness of completely melted slag, the remainder of the bath being covered with a layer some two or three inches thick of mushy, partly fused slag. If the fluorspar content be increased much above 20% or if more than a trace of silica or silicate be present the fusibility and mobility of the slag will be so increased that the craters will extend entirely through the slag thereby bringing the arc into contact with the metal which is fatal to success.

The resulting alloy will have slightly less chromium and molybdenum than the charge would indicate, owing to slag losses, but if carefully performed will have very little added carbon. We have suggested herein the use of standard materials of the least expensive commercial grade which will do the work. Ferrochrome and ferromolybdenum of lower carbon content can be purchased but need not be employed if the melting is done as herein outlined, whereas if this process is not followed it makes very little difference what grade of material is employed owing to the rapid absorption of carbon.

We do not restrict ourselves to molybdenum as an added agent, since it can be replaced by tungsten or entirely omitted. Also we do not restrict ourselves to ferro-molybdenum (or ferro-tungsten) as a source, although this product is generally more easily available and is always more easily dissolved.

While we do not restrict ourselves to any one deoxidizing agent, we have had excellent results with a mixture of cerium, magnesium, and aluminum, cerium constituting about 5% of such mixture and the entire mixture amounting to about 1/10 of 1% of the entire charge. Also while we do not restrict ourselves to any one added component we have had excellent success with molybdenum added in the form of ferromolybdenum, which is cheaper and more easily dissolved than pure molybdenum.

If the slag tends to become thin and the craters to break through, more lime is added;

if it becomes too refractory the fluorspar content is increased. Not only are carbon and silica excluded from the bath but also from all tools and from the metal contacting surfaces of moulds in which the castings are made. The best plan we have discovered is to line the molds with magnesite which can easily be done by sifting some of the finely ground material upon the patterns prior to adding the molding sand. This lining should also extend through the sprue-hole.

In magnesite molds the alloy, when made as herein described, produces smooth, solid, homogenous castings having a tensile strength of from 27,000 to 60,000 lbs. per square inch, and a Brinnell hardness of about 300 to 250. Such castings possess a true, solid-solution condition and a dense, closely-knit, uniform, crystalline structure. Such an alloy shows no corrosion by 10% solutions of nitric or sulphuric acid at room temperature after 120 days, is absolutely immune to caustic solutions, and is scarcely attacked by hydrochloric acid.

So far as our improved process is concerned we do not restrict ourselves to the compositions of matter herein described since our process is applicable to numerous other alloys which are desired to be produced in a carbon free state, especially alloys containing chromium.

So far as concerns the manufacture of apparatus we claim our composition as a new and valuable alloy not heretofore known or used. We do not, however, restrict ourselves to any details, either of apparatus, composition, or manipulation except as recited in the claims hereto annexed.

Having thus described our invention what we claim is:

1. The process of preparing alloys of chromium with one or more iron group metals which contains the steps of first melting the iron group metal or metals in an electric arc furnace, second covering the molten iron group metal with a carbon-free slag which is electrically conducting at elevated temperatures and is sufficiently basic and refractory to prevent the arc from striking therethrough, and third dissolving the chromium content in the molten iron group metal.

2. A slag for chromium containing alloys containing upwards of 80% of lime and 10% of fluorspar and substantially free from carbon and silicon or compounds thereof.

3. A slag for chromium containing alloys consisting of about 80% to 90% of lime and 20% to 10% fluorspar.

In testimony whereof, we hereunto affix our signatures.

WILLIAM H. SMITH.  
CHARLES M. CAMPBELL.